

# UNITED STATES PATENT OFFICE.

WINFIELD S. POTTER, OF NEW YORK, N. Y.

MANUFACTURE OF MANGANESE STEEL.

968,602.

No Drawing.

Specification of Letters Patent. Patented Aug. 30, 1910.

Application filed June 18, 1910. Serial No. 567,696.

To all whom it may concern:

Be it known that I, WINFIELD S. POTTER, a citizen of the United States, residing in the city and State of New York, and whose post-office address is 30 Church street, New York city, New York, have invented certain new and useful Improvements in the Manufacture of Manganese Steel; and I do hereby declare the following to be a full, clear, and exact description of the invention, such as will enable others skilled in the art to which it appertains to make and use the same.

In an application for Letters Patent of the United States, filed by me under date of May 20, 1910, Serial No. 562,374, I have described and claimed the production of a manganese steel ingot, devoid of dendrites and other objectionable freezing structures and of a strong uniform fine grained structure throughout by a series of steps beginning with the treatment of the molten metal itself before the ingots are cast, and continuing with the subsequent reconstruction of the ingot desirable for adapting it to successful commercial rolling, forging or shaping.

As broadly set forth in my application referred to, the fundamental discovery embodied therein was, that by suitably deoxidizing and cleansing the molten metal as described, while still in the furnace, casting ladle, or like source of supply, it is possible to standardize the subsequent heat treatment of the cast ingot, and, particularly, for steel of any given composition, to practically eliminate variations in that part of the heat treatment of the ingot which determines the reconstruction of the dendritic portion and its conversion into the strong uniform fine grained structure desired. The invention, as described in my said application, involved the further discovery that the preliminary deoxidation and cleansing of the metal has the function of establishing a practically definite and short period of time for the complete conversion of the dendrites and the removal of the other objectionable freezing structures, thereby enabling the operator to promptly terminate that stage of the heat treatment, which would otherwise tend to the formation and building up of large and coarse crystals or grains.

The present application, which is based upon the same fundamental features of discovery above noted, is directed specifically

to a particular method for carrying out the general operation and for realizing its characteristic advantages.

More particularly stated, this specific embodiment of the invention involves, in the general operation, the feature of preventing the formation and building up of large and coarse crystals or grains, by lowering the temperature of the outer portions of the ingot, after the objectionable freezing structures have been removed and the desired reconstruction into metal of uniform fine grain has been accomplished.

It also includes the further feature of supplementing this lowering of the temperature of the outer portions of the ingot for the purpose described, with the additional step of lightly working the ingot, so as to form a tough thick skin thereon, before it is subjected to subsequent heavy reduction; the ingot, cleansed of its oxids by the preliminary treatment of the metal in the furnace, ladle or the like, and brought to the uniform fine grained condition in its outer portions, being especially adapted, in the condition in which it then finds itself, to receive, by light rolling, the tough thick skin contemplated.

The preliminary treatment of the metal, including the compounding thereof, is fully set forth in its preferred embodiment, in my application for Letters Patent of the United States hereinbefore referred to, wherein it is assumed that, in the particular instance given, the manganese steel is to be compounded from suitably dephosphorized and desulfurized open hearth steel from an open hearth furnace, and molten ferro-manganese, mixed in the desired proportions in a casting ladle of large capacity or other suitable container appropriate for the purpose. The operations of compounding the metal, deoxidizing and cleansing it, may, however, be effected in the open hearth or like furnace itself, although, in the case of this very readily oxidized metal, the most complete deoxidizing, cleansing and washing can only be secured by continuing those operations in the ladle itself and with the employment of a protective cover of acid slag, as herein-after described.

Assuming that the compounding of the metal is to be effected in the casting ladle of large capacity, (say sixty tons or more) the ladle will be lined with the usual silicious or acid lining, preheated in the customary

manner. The charge of dephosphorized molten steel from the open hearth or like furnace will then be run into the ladle and simultaneously therewith the molten ferromanganese will likewise be charged therein. 5 As the charge of molten metal rises in the ladle, it is essential for the purpose of the invention to maintain upon its upper surface a protecting layer of acid slag. For this purpose, the ladle may, if desired, be charged with a small quantity of readily fusible acid slag making materials, or a mixture which will form a readily fusible acid slag, before the steel is running from the furnace; or in 10 lieu thereof, or in addition thereto, the acid slag making material may be added from time to time to the charge, as the level of the metal rises in the ladle. The acid slag making materials may conveniently consist of 15 silica or other silicious material associated with a sufficient amount of fluxing ingredients such as sodium silicate, lime, or lead oxide, to make it readily fusible at a sufficiently low temperature, and the proportion 20 of silica should be sufficient to balance the oxids present in the steel, (as, for instance, the oxid of iron and oxid of manganese) which it is the purpose of my invention to eliminate, as far as possible, by 25 the treatment proposed. The purpose of charging the acid slag making materials into the ladle either before or during the charging of the molten steel is, furthermore, to obtain such an intimate contact of the 30 acid slag formed and the metal as to insure, to the greatest extent possible, the washing out of the oxids from the steel throughout the entire mass thereof. Usually, it will not 35 be found feasible to charge the steel from 40 the open hearth or other furnace into the ladle without likewise encumbering it with a practically unavoidable proportion of the furnace slag containing basic oxids; and, it will be understood that the amount of 45 acid slag making materials to be charged into the ladle should be sufficient to likewise balance and neutralize these basic oxids from the furnace. In fact, the quantity of acid slag making materials charged into the 50 ladle should be somewhat in excess of that required both for cleansing the steel from its contained oxids and also for balancing the oxids admitted from the furnace with the furnace slag, in order that the body of 55 slag finally floating upon the charged metal in the ladle shall be devoid of any oxidizing effect upon the charge. In charging the molten steel into the ladle it will, of course, be understood that it is preferable to avoid 60 as far as possible the entrance of any large portion of the furnace slag. This may be effected in any suitable manner, as, for instance, by diverting the slag over the side of the furnace spout into a slag receptacle. 65 Tilting furnaces may be used to advan-

tage for the production of the steel, and the opening through which the metal is discharged from the furnace will be made of such size and the furnace so tilted during the pouring operation that the steel enters 70 the ladle with but little slag, whereupon the slag may be afterward poured separately into another receptacle. After the ladle is filled, the metal with its protecting top layer of acid slag is permitted to remain at rest 75 for a period sufficient to insure the separation of the slag and metal, and is permitted to cool to the temperature desirable for casting or teeming into the ingot molds.

In order to effect an entirely satisfactory 80 cleansing of the metal in the ladle, it should be at a relatively high temperature during the cleansing operation, as compared with the temperature of final pouring into the ingot molds. For instance, the cleansing 85 operation may be carried on with the metal at a temperature of say 1400° C. to 1450° C. The metal in the ladle will preferably contain about 12% of manganese and from .80% to 1.10% of carbon; and, in order to 90 have as little piping as possible in the ingots and to permit the metal to set without undue delay in the molds, the metal in the ladle should be cooled, or permitted to cool, before the pouring operation begins, to a 95 temperature of say 1375° C. The pouring from the ladle is effected through a bottom pouring aperture, and the temperature of the metal and the attendant conditions are to be so established that the metal will set 100 in the ingot molds promptly, with the exception, perhaps, of a small proportion in the innermost longitudinal center or core of the ingot.

While the ingot is still in the mold, I 105 preferably cool it in such manner that, when stripped from the mold, the outer portions (to a depth fully including the thickness of the zone of the dendrites) will have an average temperature in the neighborhood 110 of 1000° C., (say from 950° C. to 1050° C.) except at the edges where it will be unavoidably considerably lower. This enables it to be transferred, without suffering any rupture, into a soaking pit or other like heating 11 furnace, wherein it is to be subjected to the heat treatment designed for reconstructing its exterior portions; and it also permits this heat treatment to take place without cracking the ingot. At the time of its entrance into the soaking pit or like furnace, the ingot has set and developed its freezing structures to a depth of say six inches or more inwardly from its outer skin or periphery and a zone of dendrites has formed 1 which usually occupies say about one-half of this depth. In order to break down these dendrites and to substitute therefor a strong uniform structure of fine grain, I then slowly raise the temperature of the soaking 1

pit to  $1175^{\circ}$  C. or a somewhat higher temperature (for example  $1225^{\circ}$  C.) slowly or evenly, this rise in temperature being effected in a smoky or reducing atmosphere, 5 so that the periphery of the ingot will not be oxidized. I have found that with the preliminary deoxidation and cleansing of the metal, as hereinbefore described, the breaking down of the dendrites and the substitution therefor of a strong uniform fine 10 grained structure can be accomplished at or about the temperature of  $1175^{\circ}$  C. specified, within a comparatively short period of time, say half an hour, the temperature 15 and the time of reconstruction varying somewhat with the particular composition of the metal, but within relatively narrow limits, one way or the other, from the temperature and the period of half an hour 20 referred to. I have also found that, for steel of any given composition or analysis, the preliminary deoxidizing and cleansing step permits the operator to predetermine the temperature and the time necessary for 25 the desired breaking down of the dendrites and the reconstruction of the steel. So that, not only is the period referred to shortened, but the operation as a whole is so standardized that the desired result can be anticipated with confidence. After the ingot has 30 remained at the temperature of  $1175^{\circ}$  C. or thereabout for the period necessary for the reconstruction desired, this stage of the heat treatment is arrested by lowering the temperature 35 so as to prevent the building up within the mass of larger and coarser grains. To this end, the temperature prevailing within the soaking pit or other heating furnace may be lowered by the injection of 40 water vapor, in the form of a steam jet, carrying with it water in suspension, with the result that the periphery of the ingot is reduced in temperature to say  $1100^{\circ}$  C.; or for the same purpose, the ingot may be 45 cooled by transferring it into a cooler soaking pit, for example. The lowering of the temperature of the exterior portions of the ingot is accompanied with the formation of a tough thick skin, which shrinks upon and 50 works the still plastic interior. Finally, after the cooling of the outer portions of the ingot has occurred, and the steam jet has been cut off, the outer portions of the ingot are preferably permitted to rise again in 55 temperature to say  $1125^{\circ}$  C., in order to equalize the surface temperatures and to obtain the desirable maximum ductility, whereupon the ingot may be removed from the soaking pit and is in condition to be 60 immediately rolled into rails or other products, in mills of ordinary construction. Moreover, the temperature conditions are such that a track rail, for instance, of standard length and section, rolled from such an ingot, will be delivered from the final pass 65

of the rolls at a temperature which will permit it to be toughened by quenching without being first subjected to a reheating operation.

It will be understood that the cooling temperature of  $1100^{\circ}$  C. and the reheating temperature of  $1125^{\circ}$  C. referred to are not to be regarded as absolute. They are the temperatures which are appropriate to manganese steel of what may be termed a soft analysis, that is, having, say, 1.10% of carbon, or less, whereas, when the percentage of carbon is higher, say, 1.20%, and upward, the temperature of cooling will be somewhat lower, and the temperature to which the steel may be reheated will also be lower. In other words, these temperatures will depend upon the analysis of the steel, especially with regard to its content of carbon.

As hereinbefore stated, the preliminary step of deoxidizing and cleansing the manganese steel has for its effect not only to permit the shortening and standardizing of the period in which the dendrites are broken down and converted into a uniform fine grained structure, but by clearing the metal of its oxids throughout, makes it correspondingly strong as a final product and less tender during the manipulation to which it is subjected from the time the ingot is cast until the rolling operation is completed. In addition to this, the preliminary deoxidation and cleansing of the metal and the formation thereon of a tough thick skin by the cooling to which the ingot has been subjected after its period of reconstruction, brings it into a state or condition particularly appropriate to a still further consolidation and toughening of the skin by subjecting it to light mechanical working over its periphery. This light mechanical working has the effect of imparting to the thick skin the characteristics of wrought metal, so that, when thereafter subjected to heavy reductions incident to its passage through the rolls of the mill, it will have greater ductility and the danger of rupture will be correspondingly lessened. The light mechanical working referred to will take place as a subsequent step to the cooling operation hereinbefore described, that is, immediately before the ingot (after such cooling operation) would otherwise be rolled in the ordinary mill.

The welding or consolidating of the outer portions of the ingot by the light mechanical working described is of particular importance, where the mill work immediately following is heavy and where it involves sudden reductions or rapid elongations.

In order to give a concrete instance of the light preliminary working appropriate to the practice of the invention, I will assume that the manganese steel ingot is a 20" x 20" square section. The light preliminary roll-

ing would be effected by acting first simultaneously upon two horizontal sides, and then turning the ingot and acting simultaneously upon the two remaining sides.

5 Where the analysis of the manganese steel of the ingot shows it to be low in carbon (say containing 1.10% of carbon, or somewhat less than that amount), the reduction in the first one or two passes of the preliminary light rolling may be about one inch in each pass. This first reduction along the two horizontal sides of the ingot renders the metal of those sides capable of greater elongation, and consequently, when the ingot is turned over and rolled along its opposite sides, a somewhat greater reduction can take place, say one and one-half or one and three-quarter inches. These two preliminary reducing passes will in general suffice 20 for the light preliminary rolling intended, although, in some instances, they may be supplemented by a third or even a fourth pass, if the mill conditions are such that the light preliminary rolling can be effected quickly. When the manganese steel has a harder analysis, *i. e.*, when the percentage of carbon is as high as 1.20%, or higher, it will usually be advisable to limit the first reductions of the series of light preliminary 25 passes to from one-half to three-quarters of an inch, it being permissible, however, to somewhat increase the reduction in the subsequent pass or passes, for the reason hereinbefore explained, *i. e.*, because the metal of those sides which have been subjected to the action of the reducing rolls is capable of greater elongation for the next succeeding 30 pass.

When an electric furnace is used for the making or compounding of the manganese steel, and when there is present in that furnace a considerable proportion of manganese, it is difficult to avoid the production of a large amount of manganese oxid. To 35 meet this difficulty, it will be desirable, just before the metal is tapped from the electric furnace into the ladle, to add to the furnace charge a reducing agent (such as silico-calcium, aluminum, ferro-titanium, or the like) in sufficient quantity to properly reduce the 40 oxids contained in the metal. The metal would then be charged into the ladle, as free as possible from the furnace slag. In view of the highly oxidizable character of the 45 metal, further oxidation will take place during the transfer of the metal from the furnace into the ladle, and therefore the final deoxidation, cleansing and washing of the 50 steel will proceed in the ladle as hereinbefore 55 described.

As has been hereinbefore indicated, the 60 temperature of the ingot may be raised in the soaking pit, in some instances, to a degree higher than 1175° C. in its exterior 65 portions; in fact, to somewhat exceed this

limit (say, by bringing the temperature of the exterior portions to 1225° C.) will be found useful in most instances in order to insure greater reliability in case the casting conditions should be more or less unfavorable to the operation, and in order to obtain a correspondingly greater ductility of the metal during its passage through the roll.

What I claim is:

1. In the production of manganese steel 75 ingots and their subsequent heat treatment, in order to remove their objectionable freezing structures, the preliminary step of cleansing and deoxidizing the metal from which the ingot is cast to an extent sufficient 80 to substantially eliminate variations in the temperature necessary for the reconstruction desired, subjecting the ingot to a reconstructing temperature until the objectionable freezing structures have been removed, 85 and, after such reconstruction, lowering the temperature of the outer portions of the ingot so as to avoid the production of large and coarse grains; substantially as described.

2. In the production of manganese steel 90 ingots and their subsequent heat treatment in order to remove their objectionable freezing structures, the preliminary step of cleansing and deoxidizing the metal from which the ingot is cast to an extent sufficient 95 to substantially eliminate variations in the temperature necessary for the reconstruction desired, casting the metal at a temperature but slightly above its freezing or setting point, subjecting the ingot to the reconstructing temperature until the objectionable freezing structures have been removed, and, after such reconstruction, lowering the temperature of the outer portions of the ingot 100 so as to avoid the production of large and coarse grains; substantially as described.

3. In the production of manganese steel 105 ingots and their subsequent heat treatment in order to convert their dendrites into structures of uniform fine grain, the preliminary 110 step of cleansing and deoxidizing the metal from which the ingot is cast to an extent sufficient to substantially eliminate variations in the temperature necessary for the reconstruction desired, subjecting the ingot to the 115 reconstructing temperature until the desired uniform fine crystalline structure has been produced, and, after such reconstruction, lowering the temperature of the outer portions 120 so as to avoid the production of large and coarse grains; substantially as described.

4. In the production of manganese steel 125 ingots and their subsequent heat treatment in order to convert their dendrites into structures of uniform fine grain, the preliminary 130 step of cleansing and deoxidizing the metal from which the ingot is cast to an extent sufficient to substantially eliminate variations in the temperature necessary for the

reconstruction desired, subjecting the ingot to the reconstructing temperature until the desired uniform fine crystalline structure has been produced, and, after such reconstruction, lowering the temperature of the outer portions so as to avoid the production of large and coarse grains, and finally lightly working the outer portions of the ingot so as to produce a wrought tough thick skin; substantially as described.

5. In the production of manganese steel ingots and their subsequent heat treatment, in order to remove their objectionable freezing structures, the preliminary step of 5 cleansing and deoxidizing manganese steel containing about 12% Mn and about 1% C. from which the ingot is cast, the cleansing and

deoxidation being carried to an extent sufficient to substantially eliminate variations in the temperature necessary for the 20 reconstruction desired, subjecting the ingot to a reconstructing temperature until the objectionable freezing structures have been removed, and, after such reconstruction, lowering the temperature of the outer portions of the ingot so as to avoid the production of large and coarse grains; substantially 25 as described.

In testimony whereof I affix my signature, in presence of two witnesses.

WINFIELD S. POTTER.

Witnesses:

ELSA M. GEILFUSS,  
WILLIAM H. DAVIS.